

Dec. 19, 1944.

J. C. DITTMER

2,365,177

PROCESS FOR REFINING LEAD OR LEAD ALLOYS

Filed March 19, 1942

RECOVERY OF BISMUTH FROM THE CAUSTIC SODA SLAG

BY  
(A) LEACHING OR (B) SMELTING



FIG. 1.

FIG. 2.  
BATCH OR CONTINUOUS RECOVERY OF  
BISMUTH FROM THE CAUSTIC SODA SLAG



JOSEPH C. DITTMER  
INVENTOR.

BY *John B. Henrich Jr.*

ATTORNEY

## UNITED STATES PATENT OFFICE

2,365,177

## PROCESS FOR REFINING LEAD OR LEAD ALLOYS

Joseph C. Dittmer, St. Albans, N. Y., assignor to  
 National Lead Company, New York, N. Y., a  
 corporation of New Jersey

Application March 19, 1942, Serial No. 435,294

12 Claims. (Cl. 75—78)

The present invention relates to the refining of lead and lead alloys. More particularly it relates to a process for the refining of lead or lead alloys by the removal of the bismuth contained therein to any extent desired up to the total bismuth content, and more selectively than by methods heretofore used.

It is known that bismuth may be removed from lead or lead alloys by the use of alkali and alkaline earth metals, which react with the bismuth to form intermetallic compounds having higher melting points than the base metal treated. However, such methods of removal have not been wholly satisfactory since, because of the solubility of the bismuthide in the base metal, it has not been possible to obtain a substantially complete removal of the bismuth from the lead or lead alloys.

Furthermore, the intermetallic compounds formed in such removal processes are contained in a wet metallic mush or dross which is largely composed of the base metal, i. e., the lead or lead alloy, treated.

Hence, various "drying" methods have been suggested in order to reduce the quantity of base metal held by the wet mush. However, in spite of these drying treatments, considerable base metal is still held by the dry dross.

The prior art has also suggested subsequent treatments of the wet dross by various operations or combinations of operations involving pressing, liquating, and leaching in acid solutions or in molten baths of fluxes for the purpose of lowering the lead base metal content of the dross. However, considerable lead base metal still remains and subsequent smelting or refining operations are necessary to recover these metal values.

Another recommendation of the prior art is to treat the dross containing bismuthides with water or dilute acid solutions so as to decompose the bismuthides and liberate bismuth which, it is claimed, can then be separated from the bulk of lead base metal by some form of classification. However, these treatments involve extra operations, the handling of large amounts of drosses, and the reclaiming and retreatment, with attendant losses, of a considerable amount of lead base metal associated with the bismuthides in the dross, which dross may amount to about 10% or more of the original metal treated.

Objects of the present invention include overcoming the disadvantages described above; obtaining a substantially complete, selective and inexpensive removal of bismuth from lead or lead alloys; preventing the formation of a large metal

dross which is a considerable proportion of the metal treated and which is uneconomical to rework; and recovering the bismuth which has been removed from the base metal. Further objects 5 will become apparent as the description of my invention proceeds.

My invention contemplates treating in a molten condition the lead or lead alloy containing bismuth with one or more of the alkali or alkaline earth metals, thereby to form a bismuthide. This reaction is carried out in the presence of a flux of caustic soda. Thus, I have found that by covering the molten bismuth containing base metal with a molten flux of caustic soda which will 10 dissolve the bismuthide, and, while preferably stirring the metal, gradually adding an alkali, alkaline earth intermetallic reagent such as metallic sodium, while maintaining the temperature preferably as close to the melting point of the 15 metal as practical operation will permit, the bismuth can be substantially completely and selectively removed from the lead or lead alloy base metal, and in one operation if desired. While it 20 is preferable, in order to insure a substantially complete removal of the bismuth, to employ an 25 amount of the alkali or alkaline earth metal reagent in excess of theoretical stoichiometric requirements, just sufficient amounts of flux and intermetallic reagent may be added to effect the 30 removal of the bismuth to the desired extent, and these amounts will depend upon the quantity of bismuth to be removed, and the desired completeness of the removal. It has been found that the 35 last traces of bismuth are much more difficult to remove and therefore require relatively larger proportions of flux and reagent.

For example, in removing substantially all the bismuth from a lead alloy containing about 0.1% bismuth, sufficient metallic sodium was used to bring the sodium content of the metal to about 4% Na. Only enough caustic soda to dissolve the sodium bismuthide and still maintain the slag sufficiently fluid would be necessary, but it is usually advantageous to use more in order to keep the surface of the metal covered to prevent its oxidation. The caustic soda also prevents the oxidation of metallic sodium during its addition.

The sodium can be introduced in solid form into the molten metal under treatment either as metallic sodium or as a high percentage sodium alloy 40 by methods well known to those experienced in the art. Thus, bricks of metallic sodium can be cut up into small pieces and rapidly projected in any suitable way into the vortex of the vigorously stirred base metal or, because of the lightness 45 50 55

of metallic sodium, the sodium can be cut or otherwise formed into small pieces or particles, then mixed with the desired proportion of powdered lead, pressed into the proper sized briquet and this briquet fed into the vigorously stirred base metal. Alternatively, the sodium or sodium alloy, in an atmosphere of dry nitrogen gas, can be melted in a suitable container and fed through a proper size nozzle and pipe directly into the rapidly stirred base metal.

The sodium in whatever form or way it is introduced, reacts with the bismuth contained in the lead or lead alloy forming sodium bismuthide. I have found that a relatively large excess of sodium decreases the solubility of the bismuthide in the base metal. Simultaneously, the bismuthide selectively dissolves in the molten caustic soda flux, the solubility in the flux increasing correspondingly as the solubility in the metal is decreased by the addition of the excess sodium to the metal. Thus, a very selective separation of the bismuthide from the base metal is obtained.

As an illustration of the results to be accomplished by my invention, the following example is given:

*Example No. 1*

Original metal treated: 9084 grams of an 0.109% Bi-Pb alloy.

Metal covered with molten caustic soda and stirred.

Metallic sodium added: 500 grams.

Average temperature: 342° C.

|                                                                  | Bi               | Na               |
|------------------------------------------------------------------|------------------|------------------|
| After $\frac{1}{4}$ of the sodium had been added, metal analyzed | Per cent<br>.090 | Per cent<br>1.24 |
| After $\frac{1}{2}$ of the sodium had been added, metal analyzed | .040             | 2.23             |
| After $\frac{3}{4}$ of the sodium had been added, metal analyzed | .015             | 3.42             |
| After all of the sodium had been added, metal analyzed           | .005             | 4.44             |

A comparison of the above data of Example No. 1 with that given below in Example No. 2 for a bismuth removal using four treatments with caustic soda instead of the one used in Example No. 1 shows that one treatment is sufficient to give a satisfactory removal of the bismuth.

*Example No. 2*

Original metal treated: 9072 g. of an 0.109% Bi-Pb alloy.

Metal covered with 4 successive batches of molten caustic soda.

Metal and caustic soda were stirred one hour for each treatment.

500 grams sodium: added in 4 equal portions of 125 g. each.

Average temperature: 347° C.

|                                                                   | Metal analyzed    |                 |
|-------------------------------------------------------------------|-------------------|-----------------|
|                                                                   | Bi                | Na              |
| After treatment with 1st caustic soda and $\frac{1}{4}$ of sodium | Per cent<br>0.085 | Per cent<br>1.0 |
| After treatment with 2nd caustic soda and $\frac{1}{4}$ of sodium | 0.040             | 2.25            |
| After treatment with 3rd caustic soda and $\frac{1}{4}$ of sodium | 0.0045            | 3.13            |
| After treatment with 4th caustic soda and all of sodium           | 0.0002            | 3.87            |

If desired, sodium chloride and sodium carbonate may be added to the caustic soda flux in proportions to give their respective low melting point eutectics which are of some advantage in

the bismuth removal from alloys of correspondingly low melting points.

I have found that temperatures between just above the melting points of the metal treated and the flux used and below 350° C. give the most satisfactory removals of bismuth. In the removal of bismuth from lead, temperatures of 340° to 350° C. are the most satisfactory for practical operation.

10 If desired, the slag containing the bismuthide can be skimmed off in any suitable way and leached with water to dissolve the caustic soda and break up the sodium bismuthide into sodium hydroxide and bismuth, the latter being recovered 15 by filtration and other operations well known to those experienced in the art. According to my U. S. Patent No. 1,976,333, the resulting solution of caustic soda can be used for the complete removal of the residual sodium left in the base 20 metal after the removal of the bismuth and can thus be simultaneously concentrated back again into molten caustic soda for use in the subsequent bismuth-removal treatment of other batches of bismuth-containing lead or lead alloys. The solution of caustic soda when introduced into the vortex of the vigorously stirred molten base metal gives up its moisture to act on the sodium contained therein and thus converts it into sodium hydroxide.

25 The bismuth can also be recovered from the caustic soda slag by adding silica, sand or other neutralizing materials and smelting, but this is undesirable and uneconomic.

The recovery of bismuth from the caustic soda 30 slag by either leaching or smelting in the manner above described is illustrated in the accompanying flow sheet designated as Fig. 1.

Instead of the above methods, the bismuth contained in the molten caustic soda slag can be 35 reclaimed by concentrating it in another metal. Thus, I have found that when the molten caustic soda slag containing the bismuth is vigorously stirred in contact with a molten lead or lead alloy containing little or no sodium, all the bismuth 40 can be dissolved out of the slag and goes into the lead or lead alloy. For example, 8788 grams of a lead alloy containing 0.12% bismuth and .0016% sodium was stirred for about an hour at 340° to 370° C. with 2331 grams of caustic soda 45 slag containing 0.155% bismuth and 0.08% lead. After treatment, the slag contained 0.03% lead but no bismuth, and the alloy analyzed 0.157% Bi and 0.006% Na. Most of the sodium in the slag is oxidized during the treatment and therefore 50 only some of it enters the alloy. As sodium retards the extraction by the alloy of the bismuth in the slag, it is desirable to remove the sodium from the alloy by using either a solution of caustic soda as described above or by blowing steam into the vortex of the stirred mass of metal and slag during the bismuth extraction treatment. Other methods of oxidizing the sodium can be employed such as by blowing air into the metal and slag or by adding an oxidizing reagent such as lead oxide.

I have further found that the recovery of the bismuth by the process as described in the preceding paragraph can be combined with the bismuth-removal process and thus effect economies 60 in the use of metallic sodium and caustic soda by the simultaneous and continuous operation of both processes as follows: The molten caustic soda slag in the "bismuth-removal" pot is pumped continuously during the bismuth removal treatment to the "bismuth-collecting" pot

which is preferably at a somewhat higher level and from which the slag can flow by gravity through an overflow pipe back into the bismuth-removal pot. The caustic soda slag and bismuth-collecting metal are preferably vigorously stirred in contact to effect the more rapid and efficient solution of the bismuth. The vigorous stirring also causes some oxidation of the sodium taken up by the metal, which is desirable.

The aforementioned batch or continuous method for recovering the bismuth from the molten caustic slag by concentrating the bismuth in a molten lead or lead alloy is illustrated in the accompanying flow sheet designated as Fig. 2.

It is to be understood that the foregoing description and examples of my invention have been given merely for illustrative and not limitative purposes. Therefore, it will be appreciated that there is no intention of excluding from the scope of my invention such changes and modifications as may be accomplished by the mere skill of the art.

I claim:

1. A process for removing bismuth from lead or lead alloys which comprises melting the metal to be purified, admixing therewith at least one of the metals from the group consisting of the alkali and alkaline earth metals, thereby to form a bismuthide, said reaction being carried out in the presence of a flux comprising essentially and predominantly caustic soda, which said flux is devoid of potassium hydroxide.

2. A process for removing bismuth from lead or lead alloys which comprises melting the metal to be purified, and while vigorously stirring the same, admixing therewith at least one of the metals from the group consisting of the alkali and alkaline earth metals, thereby to form a bismuthide, said reaction being carried out in the presence of a flux containing essentially and predominantly caustic soda, which said flux is devoid of potassium hydroxide.

3. A process for removing bismuth from lead or lead alloys which comprises melting the metal to be purified, and while vigorously stirring the same, admixing therewith at least one of the metals from the group consisting of the alkali and alkaline earth metals, thereby to form a bismuthide, said reaction being carried out in the presence of a flux containing essentially and predominantly caustic soda, with optional minor amounts of sodium chloride and sodium carbonate, which said flux is devoid of potassium hydroxide.

4. A process for removing bismuth from lead or lead alloys which comprises melting the metal to be purified, and while vigorously stirring the same, admixing therewith sodium to form sodium bismuthide, said reaction being carried out in the presence of a flux of caustic soda.

5. A process for removing bismuth from lead or lead alloys which comprises melting the metal to be purified, covering the same with a flux of molten caustic soda, and admixing therewith metallic sodium until the desired removal of the bismuth is effected.

6. A process for removing bismuth from lead or lead alloys which comprises melting the metal to be purified, covering the same with a flux of molten caustic soda, admixing therewith metallic sodium, and repeating the additions of flux and metallic sodium until the bismuth is substantially completely removed.

7. A process for removing bismuth from lead

or lead alloys which comprises melting the metal to be purified, covering the same with a flux of molten caustic soda, admixing therewith an amount of metallic sodium in excess of normal stoichiometric requirements, and agitating the mass at a temperature which is just above the melting point of the mass and not in excess of about 350° C., until the desired removal of the bismuth is effected.

10. 8. A process for removing bismuth from lead or lead alloys which comprises melting the metal to be purified, admixing therewith in the presence of a molten caustic soda flux, at least one of the metals from the group consisting of the alkali and alkaline earth metals, thereby to form a bismuthide, skimming off the bismuthide-containing slag formed, leaching the same with water and recovering therefrom the bismuth values.

15. 9. A process for removing bismuth from lead or lead alloys which comprises melting the metal to be purified, admixing therewith metallic sodium pieces in the presence of a molten flux of caustic soda, thereby to form sodium bismuthide, skimming off the resulting slag containing the sodium bismuthide, leaching the said slag with water, thereby to form bismuth and a caustic soda solution, recovering the bismuth and employing the caustic soda solution to remove the residual sodium which may be present in the refined metal by virtue of the bismuth removal process.

20. 10. A process for removing bismuth from lead or lead alloys which comprises melting the metal to be purified, and while vigorously stirring the same, admixing therewith in the presence of a flux of molten caustic soda at least one of the metals from the group consisting of the alkali and alkaline earth metals, thereby to form a bismuthide, skimming off the resulting bismuthide-containing caustic soda slag, stirring the said slag in molten condition with a relatively small amount of molten lead or lead alloy, substantially free of sodium, until the bismuth values are dissolved therein.

25. 11. A continuous process for removing bismuth from lead or lead alloys which comprises melting the metal to be purified, and while vigorously stirring the same, admixing therewith in the presence of a flux of molten caustic soda, at least one of the metals from the group consisting of the alkali and alkaline earth metals, thereby to form a bismuthide, continuously removing a part of the resulting molten bismuthide-containing caustic soda slag, stirring the said slag in contact with a relatively small amount of molten lead or lead alloy until the bismuth values are substantially dissolved therein and returning the resultant molten caustic soda slag for further use in the bismuth-removal treatment.

30. 12. A continuous process for removing bismuth from lead or lead alloys which comprises melting the metal to be purified, and while vigorously stirring the same, admixing sodium therewith in the presence of a flux of molten caustic soda, thereby to form a bismuthide, continuously removing a part of the resulting molten bismuthide-containing caustic soda slag, stirring the said slag in contact with the relatively small amount of molten lead or lead alloy until the bismuth values are substantially dissolved therein and returning the resultant molten caustic soda slag for further use in the bismuth-removal treatment.

JOSEPH C. DITTMER.